

1

3,157,504

**METHOD OF INHIBITING DISCOLORATION OF COLOR PHOTOGRAPHIC LAYERS CONTAINING DYE IMAGES AND RESULTING PHOTOGRAPHIC PRODUCTS**

Charleston C. Bard, Rochester, N.Y., assignor to Eastman Kodak Company, Rochester, N.Y., a corporation of New Jersey

No Drawing. Filed Apr. 2, 1962, Ser. No. 184,494  
7 Claims. (Cl. 96—61)

This invention relates to color photography and more particularly to methods for preventing discoloration of photographic dye images. The invention also includes photographic layers or elements stabilized against discoloration according to the new methods.

Photographic color images can be produced by a variety of processes. Perhaps the most common involves the formation of the desired color record by coupling between one or more color couplers and the oxidation products of an ordinary photographic color developing agent, such as a phenylenediamine. The color coupler in such processes can be incorporated either within the photographic element itself, or within the color developer solution. Another method of producing a color record involves the use of the well known dye bleach process, wherein a uniformly dyed layer is selectively bleached in accordance with a silver record produced through conventional photographic development. Bleaching occurs at the site of formation of the silver image. Still another means of producing a photographic color image is through a diffusion transfer process which uses a dye developer to effect photographic development and to produce a diffusible dye, which then migrates imagewise to a receiving surface. The present invention provides a means of stabilizing all of these types of photographic dye images, although it is particularly useful in preserving dye images which have been produced by the conventional process of color development using a color developer containing the color-forming compound, or coupler. This latter process is a reversal type of process wherein the color development is preceded by a conventional black-and-white development operation which produces a negative silver image. After negative development, there is one or more exposures followed by color development in a developer containing the desired color-forming compound, or coupler.

It is, therefore, an object of the present invention to provide an improved method for preventing the discoloration or decomposition of photographic layers containing dye images subject to fading, or print-out under the influence of actinic radiation. It is a further object to provide photographic color materials, including films, transparencies, or prints which have been stabilized by treatment with particular stabilizing compounds. Other objects will become apparent from a consideration of the following description and examples.

The foregoing objects are accomplished according to my invention by bathing the finished photographic record (i.e., after complete color-development, bleaching, fixation, etc.) with an aqueous solution containing a water-soluble  $\alpha$ -glucoheptonate salt, or the acid, *per se*. These stabilizing compounds can be represented by the following general formula:



wherein M represents a hydrogen atom or a water-solubilizing cation, such as ammonium, alkali metal (e.g., sodium, potassium, etc.), or organic ammonium (e.g., triethanol ammonium, pyridinium, etc.). These compounds may be used in the form of their hydrate derivatives, since

2

they are rather hydroscopic, or tend to spontaneously absorb water from ambient surroundings. A particularly useful treating agent is sodium  $\alpha$ -glucoheptonate dihydrate.

- 5 The system of three-color photography suggested by Fischer in U.S. Patent 1,055,155, issued March 4, 1913, forms the basis for a number of color photographic processes and products. In one embodiment, this process involves the incorporation of different color-forming coupler 10 compounds in each of three superposed differently color-sensitized (red, green and blue) silver halide emulsion layers. Each of the three couplers is capable of producing a color complementary to the sensitivity of the layer in which it is incorporated by reaction with the oxidation 15 products of certain types of photographic developing agents. In this way a developed silver image and a colored dye image are formed simultaneously in each of the three superposed emulsion layers. The silver images and residual undeveloped silver halide may then be removed 20 from the multilayer photographic element by bleaching, fixing and washing according to now well-known methods. Alternatively, the color-forming couplers can be incorporated in the developer rather than in the emulsion layers as disclosed in Fischer U.S. Patent 1,102,028, issued June 25 30, 1914.
- The couplers suggested by Fischer containing phenolic hydroxyl, or ketomethylene groups, react with the oxidation products of aromatic amine developing agents during 30 photographic development to form indophenol, indamine, indoaniline or azomethine (including quinone-imine) dyes. Dyes produced by developing with aminophenols in the presence of a phenol or naphthol coupler are indophenol dyes, those produced by developing with a phenylenediamine type developer in the presence of an aniline 35 coupler, phenol or naphthol couplers, or reactive methylene compounds are indamine, indoaniline and azomethine dyes, respectively. Azomethine and indoaniline dyes are present in many of the processed photographic color products produced by current photographic processes.
- 40 While the process of Fischer U.S. Patent 1,055,155 in which the color-forming couplers are incorporated in the emulsion layers is theoretically feasible, it has not been entirely successful due to the tendency of the couplers to diffuse out of their respective emulsion layers during coating, or processing. For this reason, it has been proposed 45 to react the coupler molecules with high molecular weight, or colloidal, bodies to render the couplers non-diffusing in gelatin or other colloidal media. It has also been proposed to mix the couplers with a water-insoluble colloid, such as a natural or synthetic resin, or a cellulose 50 ester, and to subsequently disperse this mixture in the gelatin emulsion. Methods of this type are disclosed in Martinez U.S. Patent 2,269,158, issued January 6, 1942, and in Mannes and Godowsky U.S. Patents 2,304,939 and 55 2,304,940, issued December 15, 1942. These patents also disclose specific couplers adapted to be dispersed in emulsion layers as just described. Other couplers are disclosed in Jolley et al. U.S. Patent 2,322,027, issued June 15, 1943, Fierke et al. U.S. Patent 2,801,171, issued July 30, 1957, and in Porter et al. U.S. Patent 2,369,489, issued 60 February 13, 1945, as well as in numerous other patents, which use a water-insoluble, crystallloid, high-boiling solvent for the color coupler.

Specific couplers useful in photographic color processes 65 in which the couplers are not dispersed in a water immiscible solvent are disclosed in the following representative references: Mannes and Godowsky U.S. Patent 2,039,730, issued May 5, 1936, hydroxy diphenyl couplers which form blue or blue-green dyes; Mannes and Godowsky U.S. Patent 2,108,602, issued February 15, 1938, acetocacetamides and cyanoacetamides, containing reactive 70 methylene groups, which form yellow dyes; Mannes and

Godowsky U.S. Patent 2,115,394, issued April 26, 1938, organic compounds containing the cyanoacetyl group which form red and magenta dyes; and Richey and Jensen U.S. patent application Serial No. 670,900, filed July 10, 1957, water soluble cyan, magenta and yellow dye-forming couplers.

The developing agents useful for color development of emulsion layers containing couplers of the type described above or for the development of emulsion layers in the presence of these couplers include the well-known primary aromatic amine silver halide developing agents, such as the phenylenediamines, including the N-alkylphenylenediamines and N-alkyltolylenediamines. These developing agents are usually used in the salt form, such as the hydrochloride, or sulfate, which is more stable than the amine. The p-aminophenols and their substitution products can also be used where the amino group is unsubstituted. The N-alkylsulfonamidoalkyl-p-phenylenediamine agents of Weissberger U.S. Patent 2,193,015, issued March 12, 1940, are also very useful. All of the developing agents have an unsubstituted amino group which enables the oxidation products of the developer to couple with the color-forming compounds to form a dye image.

Many indophenol, indamine, indoaniline and azomethine dyes are relatively unstable to light with the result that dye images in finished commercial color pictures have a tendency to fade, especially when subjected to intense illumination for extended periods of time. This is true whether the source of illumination is sunlight, tungsten, or fluorescent lamps. The cyan dyes are generally relatively less susceptible to fading than the other dyes commonly used in color photography. In processes in which the couplers are incorporated in the emulsion layers or in plain gelatin layers in the film, further difficulty is caused by residual unused coupler which tends to print-out as a stain, usually a yellow stain, under the influence of light especially in the high light areas of the picture. Magenta dye-forming couplers are generally more susceptible to print-out than others.

In general, two methods have been suggested to prevent discoloration of photographic layers. One of these comprises overcoating the photographic layer to be protected with a substance capable of absorbing ultraviolet light. Methods of this type are disclosed in Salminen and Allen U.S. Patent 2,632,701, issued March 24, 1953, and Edgerton and Staud U.S. Patent 2,747,996, issued May 29, 1956. The other method referred to above comprises treatment of photographic layers containing dye images with certain chemical compounds, particularly organic reducing agents or antioxidants, in order to stabilize the dye images and any residual coupler in the photographic layer. Methods of this type are disclosed in Vittum U.S. Patent 2,384,658, issued September 11, 1955, and Mackey U.S. Patent 2,579,435, issued December 18, 1951. Methods of the latter type have been found to be mostly empirical. For example, although the reducing agents of the Vittum patent are useful, others of similar reducing properties have no effect on the stability of photographic dye images. Further, many reducing compounds which might suggest themselves as stabilizing agents not only have no stabilizing properties but actually cause stain or destruction of dye images in photographic layers. It has, therefore, been difficult to find compounds having appreciable dye stabilizing or anti-print-out properties which are also free from other undesirable characteristics. Therefore, although the above and other methods have been suggested in the art for protecting colored photographic elements against discoloration due to fading or print-out, none has proven to be a complete solution to the problem and the search for new methods has continued.

The methods of the present invention for preventing the discoloration of water permeable photographic layers containing dye images comprise treating such layers with aqueous solutions of certain organic compounds in order to introduce sufficient quantities of these treating agents

into the photographic layers to inhibit fading of the dye images or print-out of any residual dye-forming coupler therein. In practice, the photographic element or layer containing the dye image, but substantially free from developed silver, silver halide and other soluble salts, is immersed in a bath comprising an aqueous solution of one of the treating agents of the invention. The photographic layer is allowed to remain in the bath until it has absorbed sufficient treating solution to inhibit discoloration. The photographic layer is then removed from the bath and allowed to dry containing the absorbed treating agent. Optionally, surplus treating solution may be removed from the surface of the photographic element or layer by means of a squeegee, rapid water rinse or other suitable means prior to drying. When a water rinse is employed, however, care must be taken not to remove absorbed treating agent from the treated layer.

As indicated above, my invention is particularly useful in stabilizing photographic color images produced by a reversal color process wherein the color-forming components or couplers are incorporated within the photographic color developer. One of the most common of these processes is known as the Kodachrome Process. Especially useful color-forming compounds or couplers which can be incorporated in color developers include the following:

#### COUPLERS PRODUCING CYAN IMAGES

5-(p-amylphenoxybenzenesulfonamino)-1-naphthol

5-(N-benzyl-N-naphthalenesulfonamino)-1-naphthol

5-(n-benzyl-N-n-valerylaminol)-1-naphthol

5-caproylaminol-1-naphthol

2-chloro-5-(N-n-valeryl-N-p-isopropylbenzylaminol)-1-naphthol

2,4-dichloro-5-(p-nitrobenzoyl-β-o-hydroxyethylaminol)-1-naphthol

2,4-dichloro-5-palmitylaminol-1-naphthol

2,2'-dihydroxy-5,5'-dibromostilbene

5-diphenylethersulfonamido-1-naphthol

1-hydroxy-2-(N-isoamyl-N-phenyl)naphthamide

1-hydroxy-2-(N-p-sec. amylphenyl)naphthamide

8-hydroxy-1-α-naphthoyl-1,2,3,4-tetrahydroquinoline

2-lauryl-4-chlorophenol

1-naphthol-2-carboxylic-α-naphthalide

1-naphthol-5-sulfo-cyclohexylamide

5-phenoxyacetamino-1-naphthol

5-β-phenylpropionylaminol-1-naphthol

Monochlor-5-(N-γ-phenylpropyl-N-p-sec.-amylbenzoyl-aminol)-1-naphthol

2-acetylaminol-5-methylphenol

2-benzoylaminol-3,5-dimethylphenol

2-α-(p-tert. amylphenoxy)n-butyrylaminol-5-methylphenol

6-{γ-4-[γ-(2,4-di-tert. amylphenoxy)butyramido]phenoxy}acetamido]-2,4-dichloro-3-methylphenol

1-hydroxy-2-[δ-(2,4-di-tert. amylphenoxy)-n-butyl]naphthamide

2-α-(p-tert. amylphenoxy)-n-butyrylaminol-4-chloro-5-methylphenol

2-(p'-tert. amylphenoxy-p-benzoyl)amino-4-chloro-5-methylphenol

2-(4'-tert. amyl-3'-phenoxybenzoylaminol)-3,5-dimethyl-1-phenol

2-phenylacetylaminol-4-chloro-5-methylphenol

2-benzoylaminol-4-chloro-5-methylphenol

2-anilinoacetylaminol-4-chloro-5-methylphenol

2-{4'-[α-(4'-tert. amylphenoxy)-n-butyrylaminol]benzoylaminol}-4-chloro-5-methylphenol

2-[4',3''-(4''-tert. amylphenoxy)benzoylaminol]benzoylaminol-4-chloro-5-methylphenol

2-p-nitrobenzoylaminol-4-chloro-5-methylphenol

2-m-aminobenzyl-4-chloro-5-methylphenol

2-acetamino-4-chloro-5-methylphenol

2-(4'-sec. amylbenzamino)-4-chloro-5-methylphenol

2-(4'-n-amyloxybenzamino)-4-chloro-5-methylphenol

2-(4'-phenoxybenzoylaminol)phenol

- 2(4"-tert. amyl-3'-phenoxybenzoylamino)phenol  
 2-[ $\alpha$ -(4'-tert. butylphenoxy)propionylamino]phenol  
 2-[ $\alpha$ -(4'-tert. amyl)phenoxypropionylamino]phenol  
 2-[N-methyl-N-(4"-tert. amyl-3'-phenoxybenzoylamino)]phenol  
 2-(4"-tert. amyl-3'-phenoxybenzoylamino)-3-methyl-1-phenol  
 2-(4"-tert. amyl-3'-phenoxybenzoylamino)-6-methyl-1-phenol  
 2-(4"-tert. amyl-3'-phenoxybenzoylamino)-3,6-dimethyl-1-phenol  
 2,6-di(4"-tert. amyl-3'-phenoxybenzoylamino)-1-phenol  
 2-[ $\alpha$ -(4'-tert. amylphenoxy)butyrylamino-1-phenol  
 2-(o-acetamido- $\beta$ -phenylethyl)-1-hydroxynaphthamide  
 2(4"-tert. amyl-3'-phenoxybenzoylamino)-3,5-dimethyl-1-phenol  
 2-[ $\alpha$ -(4'-tert. amylphenoxy)-n-butyrylamino]-5-methyl-1-phenol  
 2(4"-tert. amyl-3'-phenoxybenzoylamino)-4-chloro-1-phenol  
 3-[ $\alpha$ -(4'-tert. amylphenoxy)-n-butyrylamino]-6-chlorophenol  
 3-(4"-tert. amyl-3'-phenoxybenzoylamino)phenol  
 2-[ $\alpha$ -(4'-tert. amylphenoxy)-n-butyrylamino]-6-chlorophenol  
 3-[ $\alpha$ -(4'-tert. amylphenoxy)-n-butyrylamino]-4-chlorophenol  
 3-[ $\alpha$ -(4'-tert. amylphenoxy)-n-butyrylamino]-5-chlorophenol  
 3-[ $\alpha$ -(4'-tert. amylphenoxy)-n-butyrylamino]-2-chlorophenol  
 2-[ $\alpha$ -(4'-tert. amylphenoxybutyrylamino)-5-chlorophenol  
 2-(4"-tert. amyl-3'-phenoxybenzoylamino)-3-chlorophenol  
 5-benzene sulfonamino-1-naphthol  
 2,4-dichloro-5-benzenesulfonamino-1-naphthol  
 2,4-dichloro-5-(p-toluenesulfonamino)-1-naphthol  
 5-(1,2,3,4-tetrahydronaphthalene-6-sulfamino)-1-naphthol  
 2,4-dichloro-5-(4'-bromodiphenyl-4-sulfonamino)-1-naphthol  
 5-(quinoline-5-sulfamino)-1-naphthol

Any of the acylaminophenol couplers disclosed in Salminen and Weissberger U.S. Patent 2,423,730, dated July 8, 1947, can be used as couplers for the cyan image, e.g.



etc.

#### COUPLERS PRODUCING MAGENTA IMAGES

- 1-p-sec. amylphenyl-3-n-amy-5-pyrazolone  
 2-cyanoacetyl-5-(p-sec. amylbenzoylamino)coumarone  
 2-cyanoacetylcoumarone-5-(n-amy- $\rho$ -sec. amylsulfanilide)

- 2-cyanoacetylcoumarone-5-(N-n-amy- $\rho$ -tert. amylsulfanilide)  
 2-cyanoacetylcoumarone-5-sulfon-N-n-butylanilide  
 2-cyanoacetyl-5-benzoylamino-coumarone  
 5 2-cyanoacetylcoumarone-5-sulfondimethylamide  
 2-cyanoacetylcoumarone-5-sulfon-N-methylanilide  
 2-cyanoacetylcoumarone-5-(N- $\gamma$ -phenylpropyl)- $\rho$ -tert. amylsulfanilide  
 10 1-p-laurylphenyl-3-methyl-5-pyrazolone  
 1- $\beta$ -naphthyl-3-amy-5-pyrazolone  
 1-p-nitrophenyl-3-n-amy-5-pyrazolone  
 1-p-phenoxyphenyl-3-n-amy-5-pyrazolone  
 1-phenyl-3-n-amy-5-pyrazolone  
 15 1,4-phenylene bis-3-(1-phenyl-5-pyrazolone)  
 1-phenyl-3-acetylamino-5-pyrazolone  
 1-phenyl-3-propionylamino-5-pyrazolone  
 1-phenyl-3-n-valerylamino-5-pyrazolone  
 1-phenyl-3-chloroacetylamino-5-pyrazolone  
 20 1-phenyl-3-dichloroacetylamino-5-pyrazolone  
 1-phenyl-3-benzoylamino-5-pyrazolone  
 1-phenyl-3-(m-aminobenzoyl)amino-5-pyrazolone  
 1-phenyl-3-(p-sec. amylbenzoylamino)-5-pyrazolone  
 25 1-phenyl-3-diamylbenzoylamino-5-pyrazolone  
 1-phenyl-3- $\beta$ -naphthoylamino-5-pyrazolone  
 1-phenyl-3-phenylcarbamylamino-5-pyrazolone  
 1-phenyl-3-palmitylamino-5-pyrazolone  
 1-phenyl-3-benzenesulfonlamino-5-pyrazolone  
 1-(p-phenoxyphenyl)-3-(p-tert. amylbenzoyl)amino-  
 30 5-pyrazolone  
 1-(2',4',6'-tribromophenyl)-3-benzamido-5-pyrazolone  
 1-(2',4',6'-trichlorophenyl)-3-benzamido-5-pyrazolone  
 1-(2',4',6'-trichlorophenyl)-3-phenylacetamido-5-pyrazolone  
 35 1-(2',4',6'-tribromophenyl)-3-phenylacetamido-5-pyrazolone  
 1-(2',4'-dichlorophenyl)-3-[3'-(2'',4'')-di-tert. amylphenoxyacetamido]benzamido-5-pyrazolone  
 1-(2',4',6'-trichlorophenyl)-3-[3'-(2'',4'')-di-tert. amylphenoxyacetamido]benzamido-5-pyrazolone  
 40 1-(2',4',6'-trichlorophenyl)-3-[3'-(2'',4'')-di-tert. amylphenoxyacetamido]benzamido-5-pyrazolone  
 1-(2',4',6'-trichlorophenyl)-3-[ $\beta$ -(2'',4'')-di-tert. amylphenoxy)propionamido]-5-pyrazolone  
 45 1-(2',4',6'-triborophenyl)-3-[ $\beta$ -(2'',4'')-di-tert. amylphenoxy)propionamido]-5-pyrazolone  
 1-(2',5'-dichloro)-3-[3'-(4'')-tert. amylphenoxy)benzamido]-5-pyrazolone  
 1-(2',4',6'-tribromophenyl)-3-[3'-(4'')-tert. amylphenoxy)benzamido]-5-pyrazolone  
 50 1-(2',5'-dichlorophenyl)-3-[3'-(2'',4'')-di-tert. amylphenoxyacetamido]benzamido-5-pyrazolone  
 1-(2',4',6'-trichlorophenyl)-3-[ $\alpha$ -(4-nitrophenoxy)acetamido]-5-pyrazolone  
 55 1-(2',4',6'-trichlorophenyl)-3-(4-nitroanilino)-5-pyrazolone

#### COUPLERS PRODUCING YELLOW IMAGES

- N-amy- $\rho$ -benzoylacetaminobenzenesulfonate  
 60 N-(4-anisoylacetaminobenzenesulfonyl)-N-benzyl-m-toluidine  
 N-(4-benzoylacetaminobenzenesulfonyl)-N-benzyl-m-toluidine  
 N-(4-benzoylacetaminobenzenesulfonyl)-N-n-amy- $\rho$ -toluidine  
 N-(4-benzoylacetaminobenzenesulfonyl)-N-benzylaniline  
 $\omega$ -(p-Benzoylbenzoyl)acetanilide  
 $\omega$ -Benzoylacet-2,5-dichloroanilide  
 $\omega$ -Benzoyl-p-sec. amylacetanilide  
 70 N,N'-di( $\omega$ -benzoylacetyl)- $\rho$ -phenylenediamine  
 N,N'-di(acetoacetamino)diphenyl  
 $\alpha$ -{3-[ $\alpha$ -(2,4-di-tert.-amylphenoxy)butyramido]benzoyl}-  
 2-methoxyacetanilide  
 $\alpha$ -{3-[ $\alpha$ -(2,4-di-tert.-amylphenoxy)acetamido]benzoyl}-  
 75 2-methoxyacetanilide

4,4'-di-(acetoacetamino)-3,3'-dimethyldiphenyl  
p,p'-Di-(acetoacetamino)diphenylmethane  
Ethyl-p-benzoylacetaminobenzenesulfonate  
Nonyl-p-benzoylacetaminobenzenesulfonate  
N-phenyl-N'-(p-acetoacetaminophenyl)urea  
n-Propyl-p-benzoylacetaminobenzenesulfonate acetoacet-  
piperidine  
ω-Benzoylacetpiperide  
N(ω-benzoylacetyl)1,2,3,4-tetrahydroquinoline  
N(ω-benzoylacetyl)morpholine

In addition to the above couplers, couplers which are particularly useful in color developers include Couplers 1-64 listed in column 3-5 of Spath U.S. Patent 2,956,876, issued October 18, 1960.

The concentration of glucoheptonate in the aqueous treating solutions of the invention can range from a lower limit below which insufficient treating agent is absorbed by the treated photographic layer to provide a substantial increase in the stability of any dye image, or residual coupler therein, to an upper limit above which additional glucoheptonate has little beneficial effect. Most useful treating solutions contain from about 2 to about 20% of treating agent by weight. The optimum concentration of the treating solution varies with the particular treating agent employed, and with the particular dyes and couplers treated, as well as other factors. In general, concentrations of treating agent from about 5 to 10% are particularly useful. It should also be recognized that the nature of the photographic layer will have an effect upon the optimum concentration. For example, porous photographic elements such as photographic paper, as opposed to film, may require larger amounts of treating agent for the same degree of stabilization.

The temperature at which the treatments are carried out is not critical. As a matter of convenience, it may be desired to employ the treating solutions at room temperature. It is, of course, important that the temperature of the treating solutions should not be high enough to damage the photographic layer or element being treated, or to decompose or otherwise adversely effect the treating agent.

The treating time required in the present invention varies with the permeability to the treating solution of the photographic elements being treated. In general, a few minutes immersion in, or contact with (e.g., spraying, etc.), the treating bath is sufficient in most cases, although shorter or longer times may often be employed with success. It is, of course, essential that the photographic element be immersed long enough to absorb sufficient treating agent to provide a significant improvement in the stability of the color element against discoloration.

The invention will now be described more specifically in the following example which has been selected for purposes of illustration only and is not to be construed as limiting the scope of the invention.

#### Example

A multi-layer photographic element of the type described in Mannes et al. U.S. Patent 2,252,718, issued August 19, 1941, was exposed to an original multi-colored scene and developed for about 3½ minutes at 80° F. in a developer having the following composition:

|                                  |      |      |
|----------------------------------|------|------|
| Quadrifos <sup>1</sup>           | g--  | 0.6  |
| Sodium sulfite                   | g--  | 12.0 |
| p-N-methylaminophenol sulfate    | g--  | 5.0  |
| Sodium hydroxide                 | g--  | 1.0  |
| Hydroquinone                     | g--  | 2.0  |
| Sodium sulfite                   | g--  | 6.0  |
| Sodium carbonate                 | g--  | 35.0 |
| Potassium iodide (0.1% solution) | ml-- | 10.0 |
| Sodium bromide                   | g--  | 3.0  |
| Sodium thiocyanate               | g--  | 1.75 |
| Water to one liter               |      |      |

<sup>1</sup> Sodium tetraphosphate (or hexametaphosphate).

The photographic element was then spray washed with water for about ½ minute and given an exposure to red illumination of 1100 ft. candle seconds. The exposed material was then developed in a cyan developer having the following formula:

|                                     |      |      |
|-------------------------------------|------|------|
| Carbohydrazide                      | g--  | 3.2  |
| Quadrifos <sup>1</sup>              | g--  | 0.7  |
| Sodium bromide                      | g--  | 2.50 |
| Potassium iodide (0.1% solution)    | ml-- | 5.0  |
| Sodium sulfite                      | g--  | 10.0 |
| Sodium sulfate                      | g--  | 20.0 |
| Sodium hydroxide                    | g--  | 3.30 |
| 6-nitrobenzimidazole (1% solution,  |      |      |
| 1% sodium hydroxide)                | ml-- | 5.0  |
| p-N-benzylaminophenol <sup>2</sup>  | g--  | 0.70 |
| Coupler <sup>2</sup>                | g--  | 1.50 |
| 4-amino-N,N-diethyl-3-methylaniline |      |      |
| hydrochloride                       | g--  | 2.60 |
| Water to one liter                  |      |      |

<sup>1</sup> Sodium tetraphosphate.

<sup>2</sup> 2-(o-acetamido-β-phenylethyl)-1-hydroxy-naphthamide.

<sup>3</sup> As hydrochloride.

In place of the carbohydrazide, it was also found possible to use 4.7 g./liter of semicarbazide, 0.25 g./liter of hydroxylamine sulfate or 0.25 g./liter of hydrazine sulfate.

The photographic element was then washed for about ½ minute with water and exposed to blue light of 300 ft. candle seconds intensity and developed in a yellow color developer containing a phenylenediamine color-developing agent, such as 4-amino-N,N-diethylaniline hydrochloride and a yellow coupler, such as Coupler No. 47 from column 4 of U.S. Patent 2,956,876. The photographic element was then washed and fogged chemically by treatment with a sodium borohydride solution, as described in Henn et al. U.S. Patent 2,984,567, issued May 16, 1961. The photographic element was then developed in a magenta color developer containing a color developing agent, such as 4-amino-N,N-diethyl-3-methylaniline hydrochloride and a magenta coupler, such as Coupler No. 30 in column 4 of U.S. Patent 2,956,876.

The photographic element, processed as described above, was split in half and one-half was then immersed for one minute in a 5% aqueous solution (by weight) of sodium α-glucoheptonate dihydrate. The immersed strip was then removed from the solution, dipped once in wash water and dried at room temperature.

Each of the above strips was then given an exposure of 360,000 foot-candle-hours to tungsten illumination. Where the original densities had been 1.0, the following density loss figures were obtained for the strips after illumination:

|                 | Red  | Green | Blue |
|-----------------|------|-------|------|
| Untreated Strip | .00  | -.36  | -.31 |
| Treated Strip   | -.02 | -.19  | -.17 |

In a similar manner, color prints of the kind referred to in "Principles of Color Photography" by Evans, Hanson and Brewer, 1953, page 307, prepared from 3 layers of light-sensitive silver halide emulsion containing, respectively, prior to color development, color couplers producing yellow, magenta and cyan dyes, and coated on a paper support, were treated with an aqueous solution containing 5% by weight of sodium α-glucoheptonate dihydrate. After the prints were thus treated, they were squeezed and dried to produce prints which showed unusual resistance to fading by actinic radiation.

If desired, a buffering agent, such as sodium tetraphosphate can be added to the stabilizing solution. Metal sequestering agents, such as ethylenediamine tetracetic acid tetrasodium salt can be added to eliminate iron staining.

As indicated above, treatment of the processed photographic color elements should be made in such a manner that a significant quantity of the glucoheptonate remains in the finished photographic color element in order to secure the desired stabilization of the dye image, or residual coupler, if this remains in the element. The optional rapid water washing of the materials treated according to the invention, should be carried out in such a way that only surplus glucoheptonate is removed from the surface of the element, and a sufficient amount of this chemical remains within the finished photographic element.

The invention has been described in detail with particular reference to preferred embodiments thereof, but it will be understood that variations and modifications can be effected within the spirit and scope of the invention as described hereinabove and as defined in the appended claims.

What I claim as my invention and desire secured by Letters Patent of the United States is:

1. A method of inhibiting discoloration of a photographic element which has been exposed, processed to a photographic record comprising at least one dye image, and residual silver and silver salts removed from the element which comprises imbibing in said processed element and aqueous solution comprising a water-soluble glucoheptonate.

2. A method of stabilizing a photographic color element which has been processed to a visible record by a reversal processing technique wherein the color-forming components are incorporated within a photographic color

20  
25  
30

developer, and residual silver and silver halide are removed from the element, comprising imbibing in said completely processed photographic element an aqueous solution comprising a water-soluble glucoheptonate.

3. A process according to claim 2 wherein said glucoheptonate is an alkali metal salt of  $\alpha$ -glucoheptonic acid.

4. A process according to claim 3 wherein said alkali metal salt is the sodium salt.

5. A method of stabilizing the dye image of a photographic element comprising a support and a plurality of photographic emulsion layers wherein said dye image comprises a dye selected from the class consisting of azomethine dyes, indoaniline dyes, indophenol dyes and indamine dyes, comprising dispersing throughout said dye image an aqueous solution containing a water-soluble glucoheptonate.

6. A process according to claim 5 wherein said glucoheptonate is an alkali metal salt of  $\alpha$ -glucoheptonic acid.

7. A process according to claim 6 wherein said water-soluble salt is sodium  $\alpha$ -glucoheptonate dihydrate.

#### References Cited in the file of this patent

#### UNITED STATES PATENTS

|           |                    |                |
|-----------|--------------------|----------------|
| 2,214,216 | Webster            | Sept. 10, 1940 |
| 2,384,663 | Weissberger et al. | Sept. 11, 1945 |
| 2,515,122 | Harsh et al.       | July 11, 1950  |
| 2,543,181 | Land               | Feb. 27, 1951  |
| 2,656,272 | Gunther            | Oct. 20, 1953  |
| 2,852,372 | Morse              | Sept. 16, 1958 |